

## UNITED STATES PATENT OFFICE

1,929,225

## ACETYL-CELLULOSE PLASTIC

James F. Walsh, East Orange, and Amerigo F. Caprio, Newark, N. J., assignors to Celluloid Corporation, a corporation of New Jersey

No Drawing. Application October 8, 1927  
Serial No. 225,016

4 Claims. (Cl. 18—48)

The practice heretofore has been to mix the cellulose acetate with sufficient plasticizer and liquid solvent to make the composition of a dough-like consistency workable in a kneader 5 or pair of rolls. This required about 60 to 100 parts of liquid solvent to the hundred of acetate, also sufficient plasticizer for the desired degree of final hardness or moldability. The gelatinous mixture is allowed to soak in a warm room for a 10 day or so and is then filtered under heavy pressure. This process of solution and manipulation has peculiar disadvantages in that the completed product, say planed sheeting, is of somewhat inferior strength or tenacity and more or less liable 15 to contain dirt and undissolved fiber which persist in spite of repeated filtering operations.

According to our invention, which is the result of many attempts to secure an acetyl-cellulose plastic comparable with one made of pyroxylin, 20 or even excelling it, we get better conversion in the dissolving and solidifying operations, with resultant strength and tenacity of superior character, also perfect freedom from dirt and undissolved fiber, by substituting the flow process 25 of conversion for the first stages of prevailing operations.

To accomplish this we dissolve the acetyl cellulose in enough liquid solvent, say 350 to 450 parts, to make a mass flowable in the cold as 30 distinguished from the usual dissolving which employs so little solvent that heat or warmth and mechanical means are required for a positive change of shape in the mass. In other words, our first stage of mixture is a so-called dope sufficiently liquid to be spread on surfaces with a 35 scraper to form thin films, whereas the usual primary stage of mixing produces a mere dough or stiff paste.

The first effect of our abundant use of solvent 40 is an almost complete conversion of the acetate fiber—a conversion unattainable when operating with doughlike solutions in a kneader or on rolls. A second effect comes from the semi-liquid condition of our mixture, which condition makes it 45 so susceptible to straining that the insolubles are held back completely and are not disposed to pass through the filter cloth like similar particles in the usual doughlike masses.

Having attained good conversion and cleanliness we reduce our flowable solution of the acetate to a condition suitable for manipulation 50 in rolls and presses to form a solid material. To secure this effect we may in some cases employ a so-called vacuum kneader or other means 55 of evaporation, but in practice we have found

the film wheel apparatus preferable, for it accomplishes solvent recovery without hazard to 60 paleness of hue and furnishes the evaporated product in a handy form. In fact, such are the peculiar advantages of the film process as a step 65 in our operations that its effect extends in a certain degree to the manipulation of solutions of pyroxylin as well as those of the acetate. Our film is not always removed from the wheel in the same condition of dryness, for the reduced 70 solvent content must correspond to the requirements of the next operations—those of coloring and solidification. If, for example, the product is to be colored or given a special shaping in rolls the solvent content will correspond in 75 some degree to that of the dough-like masses of the usual process at the roll stage, allowance of course being made for the more adaptable condition of our mixtures. For having received a superior conversion by means of our liquid 80 method, the film product does not need the usual smoothing and evening-up work but is ready for quick manipulation. Hence at this point our residual proportion or contact of liquid solvent is appreciably less than that required for 85 rolling the cellulose acetate mixtures prepared by the dough method. To give exact proportions would be uninstructive except for a particular instance. The experienced operator ascertains the proportions for himself, merely associating definite figures with definite conditions and purposes; as, for example the viscosity of his 90 acetyl-cellulose, the influence of the plasticizer, and the required time of exposure to the air when adding colors or shaping certain configurations. Many colors can be combined with our mixtures while said mixtures are still in flowable condition. This applies particularly to dyes. But in general we prefer the addition of 95 color or pigment at the rolls, or if the amount is large, and requires much mixing, as in the case of dense white, we use kneaders, in which event the amount of residual solvent must be suited to kneader action requirements. In a 100 case of heavy pigmentation, such as the one just mentioned, it is sometimes well to combine the pigment with the flowable mixture by kneader action before proceeding to recover the excess solvent either in the same apparatus or by transfer to film-wheel mechanism. Our experience, 105 however, has demonstrated that even such pigments as zinc oxide in copious proportions can be combined with the dope in the usual dope mixing tanks and that subsequent filtration perfects the combination.

After the roll operation our mixtures are prepared for the making of sheets or other form by subjection to the usual solidification operations attained by mechanism which employs heat and pressure. The essential feature of our invention is the formation of a flowable dope mixture which is readily and efficiently filtered, and which, because of such a state, gives a finished product of improved strength and uniformity of structure.

Our enhancement of strength in acetyl-cellulose products constitutes an important advance in the art and we accomplish this and freedom from impurities by means developed through much experimentation. Our preferred process has such unique features that it is applicable to the making of nitro-cellulose compounds as well as acetyl-cellulose, for it improves their cleanliness and strength in much the same manner.

20 We claim:—

1. The manufacture of a plastic substance which comprises dissolving cellulose acetate in such a large amount of solvent as substantially to complete the conversion of the cellulose acetate fibre to form a solution that can be readily filtered, filtering the solution while in a condition so nearly approaching liquidity that substantially all impurities and other insoluble materials are held back, stiffening the solution by removal of part of the solvent until a consistency suitable for roll manipulation is obtained, then working the material between heated malaxating rolls, and then subjecting the material to an operation to complete the solidification thereof.

35 2. The process of making a plastic substance which comprises dissolving a cellulose ester in

a suitable amount of volatile solvent so as substantially to complete the conversion of the cellulose ester to form a solution that may be readily filtered, filtering the solution while in a condition so nearly approaching liquidity that impurities are readily removed, forming it into partly dry films by casting the solution on a surface and causing part of the volatile solvent to evaporate, then working the films between heated rolls to remove further quantities of volatile solvent, and finally subjecting the resulting material to heat and pressure to solidify it.

3. The process of making a plastic substance which comprises dissolving cellulose acetate in a sufficient amount of volatile solvent to form a freely flowing solution, subjecting the solution to a thorough filtration to remove the undissolved impurities, forming partly dry films from such solution by casting the same on a surface and causing part of the volatile solvent to evaporate, adding color or pigment to the partly dry films, and then working the films between heated rolls to remove further quantities of volatile solvent.

4. The process of making a plastic substance which comprises dissolving cellulose acetate in a sufficient quantity of volatile solvent to form a flowable solution, subjecting the solution to a thorough filtration to remove the undissolved impurities, forming the same into partly dry films by flowing or spreading the solution and causing part of the volatile solvent to evaporate, massing the films, and then subjecting the massed films to manipulation or solidification operations by rolling, pressing or equivalent formative steps.

110  
JAMES F. WALSH.  
AMERIGO F. CAPRIO.

40

115

45

120

50

125

55

130

60

135

65

140

70

145

75

150